

July 15, 1947.

K. M. HUSTON ET AL

2,424,173

## ELECTROLYTIC PRODUCTION OF ALLOY COATINGS

Filed April 29, 1942



## UNITED STATES PATENT OFFICE

2,424,173

ELECTROLYTIC PRODUCTION OF ALLOY  
COATINGS

Kenneth M. Huston and Vincent A. Rayburn,  
Baltimore, Md., assignors to Western Electric  
Company, Incorporated, New York, N. Y., a  
corporation of New York

Application April 29, 1942, Serial No. 440,948

9 Claims. (Cl. 204—28)

1

This invention relates to electrolytic production of alloy coatings and more particularly to methods of electrolytically coating continuous lengths of metallic material with a non-ferrous alloy coating.

In the manufacture of electric conductors, it has been found to be highly desirable to brass plate conductors in order to cause outer coverings of vulcanized rubber to adhere firmly thereto. Heretofore, such brass coatings have been applied by making the conductors cathodes while passing them through an electrolyte in which solid rods, bars or plates made of a brass alloy were employed as anodes. Since these solid anodes had to be made up especially for this purpose, the cost of the brass coating was relatively high. Not only the cost, but the scarcity of the metal due to the great present day demand for it, has led to increased efforts to conserve metals and to employ reclaimed metals wherever possible. Further, as dissolution of the solid anodes progressed, the anode area decreased, thereby increasing the anode current density proportionately and contributing to the non-uniformity of plating conditions. In addition, the corroded anodes required considerable time for removal and necessitated a shutdown of the apparatus while they were being replaced.

An object of this invention is to provide new and improved methods for the electrolytic production of alloy coatings.

One method of coating metallic articles, which embodies the invention comprises providing an electrolytic cell including a metallic container which retains an electrolyte in which the metal of which the container is made is insoluble. Divided metallic material of a predetermined composition is placed in the bottom of the container in direct contact therewith and a positive potential is applied to the container which, in turn, is transmitted to the divided metallic material and makes this material the anode of the electrolytic cell. An article to be coated is immersed in the electrolyte and made the cathode of the cell to plate it with metal anodically dissolved from the divided anode material. The composition of the metal deposit is regulated within predetermined limits by adding to the divided anode material from time to time as the electrolysis progresses, divided metallic material containing the metal

2

or metals whose amounts it is desired to increase. In order to obtain the optimum results, it is also desirable to wash the divided anode material with the electrolyte to remove therefrom the sludge formed by the impurities in the anode material which tends to cover the divided anode material and to interfere with the anodic corrosion thereof.

Other features and advantages of the invention will become apparent from the following detailed description of a specific embodiment thereof, when read in conjunction with the accompanying drawings, in which

Fig. 1 is a fragmentary side elevation of an electroplating apparatus embodying the invention, a part of which is shown in section; and

Fig. 2 is a top plan view of the apparatus shown in Fig. 1.

The invention may be practiced in connection with the apparatus disclosed in the accompanying drawings in which a plurality of conductors 10—10 are first advanced from the right toward the left, as seen in Figs. 1 and 2, through contact rolls (not shown) which carry a negative electrical potential and which may be identical with rolls 11—11. Through contact with these rolls, the conductors 10—10 are also given a negative potential. The conductors enter a container 12 through weirs (not shown) formed in the right-hand end of the container, which are similar to weirs 14—14 formed in the end 16 of the container, and leave the container through the weirs 14—14. The conductors then pass between the contact rolls 11—11 which likewise have a negative potential.

A suitable electrolyte 18 is supplied to the container 12 at a rate sufficient to maintain the level of the electrolyte considerably above the bottom of the weirs in the ends of the container. In this manner, the conductors 10—10 are completely immersed in the electrolyte 18 during their entire passage through the container 12. The electrolyte which overflows from the container 12 through the weirs falls into a collecting tank 19 and is conveyed to a reservoir (not shown) from which it is later pumped back into the container 12.

In actual practice, the conductors may be advanced through the apparatus at a rate as high as 500 feet per minute, so that a plurality of containers similar to the container 12 shown in the

accompanying drawings, is required to obtain a coating of the desired thickness.

The container 12 is given a positive electrical potential, so that a divided metallic material 20 lying on the bottom of the container 12 becomes the anode in an electrolytic cell in which the conductors 10-10 form the cathodes. The divided anode material 20 may be of any composition suitable for plating the desired coating on the conductor 10-10 and may be of any suitable size, shape or configuration. The initial composite composition of the anode material is such as to supply copper and zinc ions to the electrolyte in substantially the same proportions in which these ions are present in the electrolyte initially. In the particular embodiment of the invention now being described, the anode material is finely divided metal scrap consisting principally of brass punchings, clippings, turnings, bolts, nuts, washers and the like, with sufficient copper and/or zinc scrap of similar origin added thereto to obtain a composite anode having a composition of about 65% to 90% copper and about 35% to 10% zinc.

The electrolyte 18 is pumped from a reservoir (not shown) through a pipe 21 to distributing heads 22-22 connected thereto by branch pipes 23-23. The distributing heads 22-22 are insulated from the container 12 in any suitable manner, a very desirable arrangement being described in the copending application Serial No. 441,002, filed April 29, 1942, by V. A. Rayburn. Feed pipes 24-24 are connected to the distributing heads 22-22 and carry the electrolyte to distributing pipes 25-25, which are closed at their ends by screw caps 26-26. A plurality of apertures 27-27 are formed in the distributing pipes 25-25 so as to project rapidly moving streams of electrolyte diagonally upwardly and downwardly on alternate distributing pipes 25-25 and to create considerable turbulence in the electrolyte. Preferably all of the apertures 27-27 are on the left side of the distributing pipes 25-25, as seen in Figs. 1 and 2, and cause the rapidly moving electrolyte to carry the sludge washed off of the divided metal scrap toward the left-hand of the container 12 and out through the weirs 14-14 at that end of the tank, along with the electrolyte overflowing therethrough. The downwardly projected streams of electrolyte stir up the sludge which is on the divided anode material, while the upwardly projected streams tend to keep the sludge in suspension so that it will pass out of the container 12 through the weirs 14-14 along with electrolyte in which it is suspended. The electrolyte flowing over the weirs 14-14 is collected and purified by suitable means (not shown) before it is returned to the container 12. As the plating proceeds, the composition of the brass coatings plated upon the conductors is kept substantially constant by adding divided brass or copper or zinc, or a mixture of any two or all three of these metals, to the original divided anode material in such quantities and proportions as to maintain the concentrations of the copper and zinc ions in the electrolyte substantially constant and at substantially their initial values.

In order to more particularly describe the invention, the following specific example is given:

A plurality of lead plated bronze conductors 10-10 are advanced at the rate of 350 feet per minute through the contact rolls which impart to the conductors a negative electrical potential.

The conductors are then advanced as cathodes through an electrolyte 18 retained in three containers similar to the container 12 whose combined length is 54 feet. The containers bear a positive electrical potential which is imparted to the divided metallic material held therein making this divided material the anode. A cathode current density of approximately 40 amperes per square foot is maintained in the electrolytic cell during the plating operation. The electrolyte employed in the container comprises 9.8 ounces of copper cyanide per gallon of electrolyte, 1.8 ounces of zinc cyanide per gallon of electrolyte, and 4 ounces of free sodium cyanide per gallon of electrolyte, together with a sufficient quantity of sodium hydroxide or sodium bicarbonate to cause the pH value of the electrolyte to be substantially 11.2. The temperature of the electrolyte is maintained at about 90° F. and the anode scrap consists of approximately 80% copper and 20% zinc. Under these conditions, a brass plate having a composition of approximately 78% copper and 22% zinc is deposited upon the conductors.

The use of divided metallic anodes in electroplating conductors represents a material improvement over the prior art. In the present invention, metallic material containing noticeable percentages of impurities frequently found in brass, such as lead, may be used as the anode material and as a result, scrap metal may be employed. The composition of the brass alloy deposited upon the conductors 10-10 may be controlled within predetermined limits by adding metal scrap consisting principally of copper and/or zinc to that already in the container 12 as the electrolysis proceeds. For example, should the percentage of zinc ions in the electrolyte fall below a certain minimum, sufficient metal consisting principally of zinc is added to the container to raise the amount of zinc in the electrolyte to within the range required for plating brass of the desired composition. Should the percentage of copper ions in the electrolyte drop below the minimum amount required to plate the desired composition of brass, metal consisting principally of copper is added. Brass and combinations of brass with copper and/or zinc may be added to the anode material to regulate within predetermined limits the amounts of copper and zinc therein.

Previously the composition of a cyanide brass plating bath was usually controlled by adding the very expensive cyanide salts of copper and/or zinc to the bath, since it was impossible to alter the composition of the solid metal anodes. The regulation of the composition of the electrolyte within predetermined limits by merely adding in divided form the metal in which the electrolyte is deficient is simple, flexible, rapid and very much cheaper than adding the more costly cyanide salts. In addition, this procedure eliminates the loss of time which formerly was consumed in replacing anodes. Thus, the present process decreases the cost of controlling the composition of the bath, as well as the cost of the original anode material, while at the same time, it conserves metal which, at the present time, is extremely scarce.

A process using divided anode material is not only much cheaper than the electroplating processes disclosed in the prior art, but is better adapted to plating rapidly moving lengths of metallic strands. Due to the speed of the movement

of the conductors 10—10 through the container 12, the surfaces of the conductors are exposed to the plating of the electrolyte in each container 12 for approximately three seconds. When three containers similar to container 12 are used, the conductors are immersed in the electrolyte for a total of approximately nine seconds.

In order to obtain a coating of the desired thickness upon the conductors in this short period of time, it is necessary to maintain a high cathode current density, which results in a rapid removal of copper and zinc ions from the electrolyte. Because of the relatively small surface area of the solid anodes formerly used, the copper and zinc could not go into solution at a rate equal to that at which they were plated out of solution onto the conductors. Then too, the dissolution of the anodes decreased the anode surface area which increased the anode current density. As a result, the brass coating was non-uniform and streaky. The brass coating deposited when divided brass anodes are used is uniform, since the divided nature of the anode metal greatly increases its surface area, whereby the rate at which the anode metal will go into solution is proportionately increased. Furthermore, it is relatively easy to maintain the desired anode composition without stopping the process by adding divided anode material from time to time as the operation progresses.

It is preferable to provide means for washing the sludge from the divided anode material, because the sludge deposited upon the anode material tends to suppress the anodic corrosion thereof. By using the electrolyte to wash the sludge from the anode material, no dilution of the electrolyte occurs and, consequently, no loss in the plating efficiency of the electrolytic bath results.

What is claimed is:

1. The method of continuously electroplating a uniform brass coating upon a metallic strand, which comprises advancing such a strand as a cathode through an electrolytic cell employing an aqueous copper-zinc cyanide electrolyte of such composition as to plate a brass coating of predetermined composition upon the strand, making a mass of divided bodies composed of metal of the group consisting of brass, copper, and zinc the anode in the cell, the initial composite composition of the anode being such as to supply copper and zinc ions to the electrolyte in substantially the proportions in which these ions were present in the electrolyte initially, passing an electric current through the cell to continuously plate a brass coating upon successive increments of the moving strand, and maintaining the composition of the brass coating plated upon the strand substantially constant by adding divided bodies composed of metal of the group consisting of brass, copper, and zinc to the divided anode bodies as the plating progresses in such quantities and proportions as to maintain the concentrations of the copper and zinc ions in the electrolyte substantially constant and at substantially their initial values.

2. The method of continuously electroplating a uniform brass coating upon a metallic strand, which comprises advancing such a strand as a cathode through an electrolytic cell employing an aqueous copper-zinc cyanide electrolyte of such composition as to plate a brass coating of predetermined composition upon the strand, making a mass of divided bodies composed of metal of the group consisting of brass, copper, and zinc the anode in the cell, the initial composite compo-

sition of the anode being such as to supply, copper and zinc ions to the electrolyte in substantially the proportions in which these ions were present in the electrolyte initially, passing an electric current through the cell to continuously plate a brass coating upon successive increments of the moving strand, maintaining the composition of the brass coating plated upon the strand substantially constant by adding divided bodies composed of metal of the group consisting of brass, copper, and zinc to the divided anode bodies as the plating progresses in such quantities and proportions as to maintain the concentrations of the copper and zinc ions in the electrolyte substantially constant and at substantially their initial values, and continuously washing the divided anode bodies with electrolyte to remove sludge therefrom by projecting a plurality of small, spaced, rapidly moving jets of the electrolyte into the mass of divided anode bodies so as to impinge directly upon the divided anode bodies.

3. The method of continuously electroplating a uniform brass coating upon a metallic strand, which comprises advancing such a strand as a cathode through an electrolytic cell employing an aqueous electrolyte having the composition of approximately 9.8 ounces of copper cyanide per gallon of electrolyte, 1.8 ounces of zinc cyanide per gallon of electrolyte, and 4 ounces of free sodium cyanide per gallon of electrolyte; making a mass of divided bodies of scrap material composed of brass and metal of the group consisting of copper and zinc the anode in the cell, the initial composite composition of the anode being approximately 80% copper and 20% zinc; passing an electric current through the cell to continuously plate a brass coating having a composition of approximately 78% copper and 22% zinc upon successive increments of the moving strand; maintaining the composition of the brass coating plated upon the strand substantially constant by adding divided bodies of scrap material composed of brass and metal of the group consisting of copper and zinc to the divided anode bodies as the plating progresses in such quantities and proportions as to maintain the concentrations of the copper and zinc ions in the electrolyte substantially constant and at substantially their initial values; and continuously washing the divided anode bodies with the electrolyte to remove sludge therefrom by causing a plurality of small, rapidly moving jets of the electrolyte to impinge directly upon the divided anode bodies, said jets being directed in one general direction but alternately upwardly and downwardly whereby a turbulent stream of the electrolyte is produced.

4. The method of continuously electroplating a uniform brass coating upon a metallic strand, which comprises advancing such a strand as a cathode through an electrolytic cell employing an aqueous electrolyte having the composition of approximately 9.8 ounces of copper cyanide per gallon of electrolyte, 1.8 ounces of zinc cyanide per gallon of electrolyte, and 4 ounces of free sodium cyanide per gallon of electrolyte; making a mass of divided bodies of scrap material composed of brass and metal of the group consisting of copper and zinc the anode in the cell, the initial composite composition of the anode being approximately 80% copper and 20% zinc; passing an electric current through the cell to continuously plate a brass coating having a composition of approximately 78% copper and 22% zinc upon successive increments of the moving

strand; and maintaining the composition of the brass coating plated upon the strand substantially constant by adding divided bodies of scrap material composed of brass and metal of the group consisting of copper and zinc to the divided anode bodies as the plating progresses in such quantities and proportions as to maintain the concentrations of the copper and zinc ions in the electrolyte substantially constant and at substantially their initial values.

5. The method of continuously coating metallic strands, which comprises advancing a metallic strand as a cathode through an electrolytic cell including an aqueous brass plating electrolyte, mixing divided scrap composed of brass and metal of the group consisting of zinc and copper in such proportions as to provide a composite composition of from about 65% to about 90% copper and from about 35% to about 10% zinc, making the divided scrap material the anode in the cell, passing an electric current through the cell to plate a brass coating of a predetermined composition upon the metallic strand, adding sufficient finely divided scrap of the group consisting of brass, copper and zinc to the anode mixture at intervals as the plating progresses to maintain substantially constant the composition of the brass plating electrolyte thereby producing a brass plating of substantially uniform composition upon the strand, and continuously supplying the brass plating electrolyte to the electrolytic cell in a plurality of small, rapidly moving jets which enter the cell at spaced points in direct contact with the divided anode material, whereby sludge is washed from the anode material.

6. The method of coating metallic strands, which comprises making such a strand a cathode in an electrolytic cell including an aqueous alkaline cyanide brass plating electrolyte, making a thin layer of divided scrap material of the group consisting of brass, zinc and copper the anode in the cell, the initial composite composition of the anode being such as to supply copper and zinc ions to the electrolyte in substantially the proportions in which these ions were present in the electrolyte initially, passing an electric current through the cell to plate a brass coating upon the strand, adding sufficient finely divided scrap material of the group consisting of brass, zinc and copper to the layer of divided anode material at intervals as the plating progresses to maintain substantially constant the composition of the brass plating electrolyte thereby producing a brass coating of substantially uniform composition upon the strand, and continuously supplying electrolyte to the cell in the form of a plurality of small, rapidly moving jets introduced at spaced points adjacent to the divided anode material so as to impinge directly upon the anode material, whereby sludge is washed from the divided anode material.

7. The method of coating metallic strands, which comprises rapidly advancing such a strand as a cathode through an electrolytic cell, causing an elongated stream of an aqueous alkaline cyanide brass plating electrolyte to pass longitudinally along the strand, making an elongated, thin layer of divided scrap material consisting of metals of the group consisting of brass, zinc and copper the anode in the cell, said metals being present in said layer in such proportions as to provide a composite brass anode of a predetermined composition, which will supply copper and zinc ions to the electrolyte in substantially the

proportions in which these ions were present in the electrolyte initially passing an electric current through the cell to plate a brass coating upon the strand, adding sufficient finely divided scrap material of the group consisting of brass, zinc and copper to the layer of divided anode material at intervals as the plating progresses to maintain substantially constant the composition of the brass plating electrolyte thereby produc-

10 ing a brass coating of substantially uniform composition upon the strand, and continuously supplying the electrolyte to the cell solely in the form of a plurality of small, rapidly moving jets introduced at spaced points adjacent to the divided anode material so as to impinge directly upon the anode material, said jets being directed in one general direction but alternately diagonally upwardly and downwardly, whereby a turbulent stream of electrolyte is produced which washes sludge from the divided anode material.

15 8. The method of continuously brass plating metallic strands, which comprises imparting a positive electrical potential to an elongated, insoluble metal container, placing a thin layer of divided scrap material consisting of brass and copper on the bottom of the container, whereby a positive potential is imparted to the divided material, causing a stream of an aqueous alkaline cyanide brass plating electrolyte of sufficient depth to cover the divided scrap material to flow over the scrap material, the initial composite composition of the anode being such as to supply copper and zinc ions to the electrolyte in substantially the proportions in which these ions were present in the electrolyte initially, continuously passing a metallic strand as a cathode through the electrolyte in the container to cause a brass plate to be deposited thereon, adding divided scrap material consisting of brass and copper to the layer of divided anode material as the plating progresses in such quantities and in such proportions as to maintain the plating conditions substantially constant, and continuously supplying the electrolyte to the container solely in the form of a plurality of small jets of high velocity introduced at spaced points near the bottom of the container so as to impinge upon the divided anode material, whereby sludge is washed from the divided anode material.

20 9. The method of continuously brass plating metallic strands, which comprises imparting a positive electrical potential to an elongated, insoluble metal container, placing a thin layer of divided scrap material consisting of brass and metal of the group consisting of zinc and copper on the bottom of the container, whereby a positive potential is imparted to the divided material, causing a stream of an aqueous alkaline cyanide brass plating electrolyte of sufficient depth to cover the divided scrap material to flow over the scrap material, the initial composite composition of the anode being such as to supply copper and zinc ions to the electrolyte in substantially the proportions in which these ions were present in the electrolyte initially, continuously passing a metallic strand as a cathode through the electrolyte in the container to cause a brass plate to be deposited thereon, adding divided scrap material consisting of brass and metal of said group to the layer of divided anode material as the plating progresses in such quantities and in such proportions as to maintain the plating conditions substantially constant, and continuously supplying the electrolyte to the container solely in the form of a plurality of small jets of

9

high velocity introduced at spaced points near the bottom of the container so as to impinge upon the divided anode material, said jets being directed in one general direction but alternately diagonally upwardly and downwardly, whereby a turbulent stream of electrolyte is produced which washes sludge from the divided anode material.

KENNETH M. HUSTON.  
VINCENT A. RAYBURN.

10

| Number     | Name         | Date          |
|------------|--------------|---------------|
| Re. 17,141 | Rosenquist   | Nov. 20, 1928 |
| 898,189    | Cowper-Coles | Sept. 8, 1908 |

5

| Number  | Country       | Date         |
|---------|---------------|--------------|
| 19,411  | Great Britain | 1906         |
| 312,600 | Great Britain | May 27, 1929 |

## FOREIGN PATENTS

10

| Number  | Country       | Date         |
|---------|---------------|--------------|
| 19,411  | Great Britain | 1906         |
| 312,600 | Great Britain | May 27, 1929 |

## OTHER REFERENCES

Principles of Electroplating and Electroforming, by Blum and Hogaboom, second edition (1930), pages 380 and 381.

Applied Electrochemistry, by Allmand and Ellingham, second edition (1924), page 358.

Modern Electroplating, special volume by The Electrochemical Society (1942), pages 87 to 99, inclusive.

Electrochemistry, by Creighton and Koehler, first edition, volume II (1935), page 149.

## REFERENCES CITED

The following references are of record in the file of this patent:

## UNITED STATES PATENTS

| Number    | Name     | Date          |
|-----------|----------|---------------|
| 1,363,186 | Merritt  | Dec. 21, 1920 |
| 1,768,358 | Harrison | June 24, 1930 |

15

15

20